

1

3,035,988

## METHOD OF FORMING FRICTION FILM ON HAND

Robert S. Cohen, Dover, Ohio, assignor to Dover Chemical Corporation, Dover, Ohio, a corporation of Ohio  
No Drawing. Filed Mar. 19, 1958, Ser. No. 722,367  
5 Claims. (Cl. 167—92)

This invention relates to a new composition prepared in form for use as a friction agent and in particular for use as a friction agent to be applied to the hands of athletes, and the like, who handle the tools of their activities and require that the grip be sure.

The rosin bag is a traditional piece of equipment generally seen at the pitcher's mound in a ball game so that the pitcher may dust his hand occasionally to make more certain of his grip on the ball. Similarly, tennis players seem to require a light application of powdered rosin to the hands to aid in making more certain of their grip. Golf players are quite meticulous about the club, stroke and other aspects of the game and in view of the fact that the nature of the stroke has much to do with the accuracy of placing the ball, a sure grip on the golf club is of fundamental importance to the game, and, accordingly, rosin has been a traditional material for use by golfers. The fundamental disadvantages of rosin or heavy metal soaps and other ingredients of that character which have found some use in the several applications mentioned, is their lack of permanence and relatively poor effectiveness. The bare hands of the athlete by perspiring seem to dislodge the rosin dust with the result that frequent renewal of the dusting must take place, and the friction effect of a fresh application of rosin is much less than that of the new compositions herein described.

It is, accordingly, a fundamental object of this invention to provide new compositions in both powdered and liquid forms suitable for use in dusting or coating the hands and like surfaces to form friction films, which materials will be characterized by their efficiency in forming friction films on the surface of the hands, and which will be of a degree of durability such that they can last for several hours during use in athletic events, and in their fundamental effect, are far superior to rosin.

It is another object of the invention to provide a friction film for application to surfaces which friction film will be waterproof and have a degree of permanence such that it cannot be washed off from the hands in an ordinary washing operation.

Other objects and advantages of the invention will in part be obvious and in part appear hereinafter.

This invention, accordingly, is involved in a novel composition consisting essentially of highly chlorinated paraffin, in finely divided form, suitable for use as a dusting powder or in a liquid suspension or solution suitable for use as a lotion, for application to the hands and like surfaces for the formation thereon of a friction film layer, which will improve the ability of the hand to grip a tool.

Paraffin is a fully saturated hydrocarbon generally considered to be a mixture of molecules having from about 18 to about 22 carbon atoms in the chain and the physical form of the paraffin may include soft varieties, such as microcrystalline waxes. In other words, the starting material for the preparation of the composition need correspond only chemically to the requirement that it be a quite heavy hydrocarbon of the order of 18-24 carbon atoms in size. I have found that when such a molecule is chlorinated to at least about 60 percent and preferably to 70 percent or more by weight of chlorine, it is converted to a solid which can be reduced to an extremely finely divided powder form, which powder is completely insoluble in water, tasteless, odorless, and

2

may be made completely free of hydrochloric acid. A specific preferred form of the chlorinated paraffin for use in preparing compositions in accordance with this invention is the chlorinated paraffin having the following specification.

Chlorine content ---- 69-70 percent, preferred; 60-theoretical limit useful.

Color:  
 10 Solid ----- Gardner 1933 Std. 6-7.  
 Powder ----- Light cream or off white.  
 Melting point (ball  
and ring method) -- 95-100° C.  
 Specific gravity (solid) 1.7.  
 Density (solid) ----- 14 pounds per gallon.  
 15 Density (apparent, of  
powder) ----- 55 pounds per cubic foot.  
 Particle size ----- 98 percent through 50 mesh.  
 Solubility ----- Soluble to vary extent in aliphatic and aromatic solvents to give clear solutions with no residue.  
 20 Water solubility ---- None.  
 Taste ----- None.  
 Odor ----- None.  
 25 Free acid (HCl) ---- None.

The chlorinated paraffin when prepared and reduced to this form by grinding is a free flowing dry powder. The following specific examples will illustrate the preferred form and formulation for the composition made in accordance with this invention wherein all ingredients are listed in parts by weight:

|                                                                         | Parts |
|-------------------------------------------------------------------------|-------|
| I. Chlorinated paraffin, 69-70 percent chlorine                         | 75    |
| 35 Diatomaceous earth                                                   | 25    |
| II. Chlorinated paraffin                                                | 50    |
| Diatomaceous earth                                                      | 40    |
| Magnesium oxide                                                         | 5     |
| Zinc stearate                                                           | 5     |
| 40 III. Chlorinated paraffin                                            | 90    |
| Colloidal silica gel                                                    | 10    |
| IV. Chlorinated paraffin, finely divided (50<br>mesh)                   | 100   |
| 45 V. Chlorinated paraffin                                              | 50    |
| Rosin                                                                   | 50    |
| VI. Chlorinated paraffin, finely divided                                | 50    |
| Water                                                                   | 49.4  |
| 50 Dispersing agent (Monoperse A, a lecithin)                           | .6    |
| VII. Chlorinated paraffin                                               | 20    |
| Solvent methyl ethyl ketone                                             | 80    |
| 55 VIII. Chlorinated paraffin                                           | 35    |
| Solvent methyl ethyl ketone                                             | 15    |
| Emulsifier                                                              | 5     |
| Water                                                                   | 45    |
| 60 VIII. (a) The formula of Example VIII may be<br>modified as follows: |       |
| Chlorinated paraffin                                                    | 30    |
| Solvent (methyl ethyl ketone)                                           | 15    |
| Triethanolamine                                                         | 3     |
| Oleic acid                                                              | 7     |
| Water                                                                   | 45    |

The statement of proportions in Examples I-VIII identifies preferred amounts. Actually, variations from these are acceptable if the basic principle of keeping in suspension or solution an amount of chlorinated paraffin which will produce a useful result is followed. Since solutions are viscous, they can be made with extra solvent to render them less so, i.e., the amount of extender serving as sol-

vent, there being as much as 80-90 percent in some cases.

In formulating the dry compositions, all ingredients are carefully mixed in the above dry state, care being taken to see that the state of subdivision is at least 50 mesh. In formulating a liquid such as VI, a relatively coarsely ground, highly chlorinated paraffin may be milled with water in the presence of a small amount of a dispersing agent, such as a lecithin until a smooth dispersion results.

Where desired the aqueous dispersion like VI may be prepared with smaller amounts of water and dried to form a chalk-like cake, which when rubbed on the hands forms a chalk-like film, which virtually immediately forms the friction coating.

The solution of VII is formed by simple dissolving of the chlorinated paraffin resin in an appropriate solvent, methyl ethyl ketone being typical.

The emulsion of VIII is formed by first forming the solution of chlorinated paraffin in solvent, such as petroleum ether, ligroin, benzene, toluene, etc., and adding to this the emulsifier. To the hydrocarbon solution, water is added with stirring slowly at first. When the initial emulsion of water in hydrocarbon inverts to an emulsion of hydrocarbon in water, the mixture being rapidly diluted to the desired strength.

A wide variety of ionic, anionic, cationic, and nonionic emulsifiers and couplers are available which may be used to disperse, emulsify or couple solutions of chlorinated paraffin and solvents with water.

In preparing dry compositions, attention should be given to maintaining the chlorinated paraffin in free flowing condition, because the usefulness of the material is dependent upon the user's being able to dust a small quantity onto the hand, or area, to have the film form on it. In general, an inert carrier may be mixed with the chlorinated paraffin as an extender to assist in giving it free flowing qualities or at least preserving them as well as to give bulk to the desired useful extent. Typical extenders may be noted to be diatomaceous earth, a useful variety being that sold under the trade name Microcel; colloidal silica gel, in the fluffy dry form; or magnesium oxide in anhydrous form; zinc oxide in anhydrous form; as well as anhydrous powders of heavy metal soaps, such as zinc stearate, which has certain antiseptic values.

The fundamental ingredient in the composition is the chlorinated paraffin and preferably the chlorine content of the paraffin should be about 69 to 70 percent, although paraffins having as little as 60 percent chlorine are solid and subject to being prepared in the requisite finely divided form to make them useful for the purpose. The chlorinated paraffin in the composition should be at least about 50 percent and where it has been prepared in an anhydrous condition and finely divided (a characteristic preparation shows 98 percent will pass a 50 mesh sieve) the chlorinated paraffin may be used as such without an extender to give the maximum anti-slip effect.

The carrier, in addition to totally inert filler, may include a smaller proportion of such compounds as zinc oxide or magnesium oxide for their antiseptic value. Essentially, it is to be noted from the examples, however, that the composition is characterized by its containing a large proportion of chlorinated paraffin.

The effectiveness of the composition when applied

to the hands is quite unusual in that it has an apparent affinity for the skin which is unexpected. Actually the melting point of the solid chlorinated paraffin is of the order of 70°-100° C. so that its action in forming the waterproof friction film on the skin is quite surprising, because it cannot be attributed to the melting of the compound by body heat. A reasonable mechanism for the action of the chlorinated paraffin on the hands would be to postulate the presence of some minor amounts of less highly chlorinated paraffin, hence of lower melting point, in the fully chlorinated product so that when the finely divided powder or chlorinated-paraffin containing lotion is rubbed over the hands, the less highly chlorinated material softens and induces the adhesion of the highly

chlorinated product to the skin. This is a reasonable mechanism in that when the material is rubbed over the surface of the hands, the full friction effect is not evident immediately. In the use of the liquid compositions, the solvents and diluents must be given time to evaporate. That is, it takes a short time after application (less than a minute) to develop the full friction effect.

In use by golfers, tennis players, and baseball players, it has been found that the single dusting or coating of the hands thoroughly rubbed onto the surface at the commencement of a contest or a match, has provided the user with a more than adequate friction treatment of the hands to last through the entire contest, and indeed will even continue to be effective after the hands are washed with soap and water.

Though the invention has been described with reference to only a limited number of examples, it is to be understood that variants thereof may be practiced without departing from its spirit or scope.

What is claimed is:

1. A method of forming an adherent friction film on a human hand which cannot be readily removed by washing comprising applying to said hand a composition comprising a chlorinated paraffin containing at least approximately 60% of chemically combined chlorine.
2. A method as defined in claim 1 wherein said paraffin contains 18 to 22 carbon atoms.
3. A method as defined in claim 1 wherein said paraffin contains at least approximately 70% of chemically combined chlorine.
4. A method as defined in claim 1 wherein said composition is in the form of a finely divided powder.
5. A method as defined in claim 4 additionally comprising sufficient dry colloidal silica to increase the ability of the composition to flow freely.

#### References Cited in the file of this patent

#### UNITED STATES PATENTS

- |           |              |               |
|-----------|--------------|---------------|
| 2,640,366 | Knuth -----  | June 7, 1953  |
| 2,819,681 | Luvisi ----- | Jan. 14, 1958 |

#### FOREIGN PATENTS

- |         |                   |               |
|---------|-------------------|---------------|
| 257,406 | Switzerland ----- | Mar. 16, 1949 |
|---------|-------------------|---------------|

#### OTHER REFERENCES

- 60 Warth: "The Chemistry and Technology of Waxes," pub. 1956, by Reinhold (pp. 450-451).

- Condensed Chemical Dictionary, 4th ed., pub. 1950, Reinhold (p. 286).